# EUROPEAN PATENT SPECIFICATION

(11) **EP 4 201 229 B1**
(45) Date of publication and mention of the grant of the patent: **19.06.2024**
(21) Application number: 22214279.6
(22) Date of filing: 16.12.2022
(51) Int. Cl.: A24B 15/16, A24B 15/14, A24B 15/167, A24B 15/30, A24B 15/18

(54) **A METHOD FOR PREPARING A HOOKAH CONSUMABLE COMPOSITION**
VERFAHREN ZUR HERSTELLUNG EINER VERZEHRBAREN HOOKAH-ZUSAMMENSETZUNG
PROCÉDÉ DE PRÉPARATION D'UNE COMPOSITION CONSOMMABLE DE NARGUILÉ

(30) Priority: 23.12.2021 NL 2030265
(43) Date of publication of application: 28.06.2023
(73) Proprietor: HTL-DHT B.V., 5642 JA Eindhoven (NL)
(72) Inventor: WIJERS, Steven Dirk, EINDHOVEN (NL)
(74) Representative: Algemeen Octrooi- en Merkenbureau B.V.

(56) References cited:
- EP-A1- 3 351 121
- EP-A1- 3 442 363
- EP-B1- 3 442 363
- WO-A1-2020/012761
- WO-A1-2020/044179
- WO-A1-2020/235112
- WO-A1-2021/122583
- WO-A1-2021/170670
- CN-A- 110 236 218
- DE-U1-202020 002 254
- US-A- 3 965 911
- US-A- 4 333 484
- US-A1- 2018 199 617
- US-A1- 2019 328 030
- US-A1- 2021 259 307

## Description

The present invention relates to a method for preparing a hookah consumable composition. The present invention also relates to the use of such a hookah consumable composition.

### FIELD OF THE INVENTION

Shisha may refer to a water pipe, or product consumed in a water pipe. In the context of this application, shisha refers to the product consumed in a hookah or water pipe. Hookahs are traditionally used to smoke shisha tobacco and are configured such that vapour and smoke pass through a water basin before inhalation by a consumer. Typically, the shisha tobacco is placed in a cup which sits on top of a water container. This cup is connected to a pipe of which the other open end is submerged in the water in the container. The cup is sealed with a perforated lid or tin foil. The shisha tobacco is heated by placing hot pieces of charcoal on top of the sealed cup. On the sides of the water container, one or more tubes are connected. The consumer inhales through the tube, which draws the vapours from the heated tobacco through the water to the consumer. Shisha devices may include one outlet or more than one outlet so that the device can be used by more than one consumer at a time. Use of shisha devices is considered by many to be a leisure activity and a social experience. The composition used in shisha devices may be mixed with other ingredients to, for example, increase the volume of the vapour and smoke produced, to alter flavour, or both. Charcoal pellets are typically used to heat the tobacco in a shisha device, which may cause full or partial combustion of the tobacco or other ingredients. Some shisha devices have been proposed that use electrical heat sources to, for example, avoid by-products of burning charcoal or to improve the consistency with which the composition is combusted. Other shisha devices have been proposed that employ e-liquids. A hookah session is meant to be a relaxing and often social event where people come together. A typical hookah session can usually be between 20 and 90 minutes.

EP 3 442 363 relates to a shisha consumable article for use with a shisha assembly, the shisha consumable article, comprising: a housing defining a first compartment and a second compartment, the second compartment being adjacent to, and sealed or air impermeable from, the first compartment; a combustible heat source contained within the first compartment; and an aerosol-forming substrate contained within the second compartment. The aerosol-forming substrate includes nicotine or a nicotine source, wherein the nicotine comes from tobacco leaf material.

WO 2020/044179 relates to a shisha cartridge comprising: a body comprising a cavity and an internal cavity surface; an aerosol-forming substrate disposed in the cavity; an absorbent carrier disposed in the cavity; and an aerosol former impregnated into the absorbent carrier, wherein the aerosol former comprises glycerine, propylene glycol, or a combination thereof, wherein the absorbent carrier comprises refined cellulosic material, i.e. paper.

US 2019/328030 relates to a method of making a nicotine containing sheet, comprising combining a source of nicotine salt having a cellulose content of less than about 5% by weight on a dry weight basis with a separate source of fibrous material having a nicotine salt content of less than about 5% by weight on a dry weight basis to form a mixture; and drying the mixture to form a sheet.

WO 2020/235112 relates to an aroma-producing body to be heated loaded into an aroma cartridge comprising an aroma-producing substrate to be heated, the aroma-producing substrate to be heated producing smoke and aromas when heated in contact with a heating element; and a packaging material rolling up the aroma-producing substrate to be heated, wherein the aroma-producing substrate to be heated includes at least an aerosol former, non-tobacco plants and/or tobacco plants, and a binding agent.

WO 2021/170670 relates to an aerosol-generating article comprising an aerosol-generating substrate, the aerosol generating substrate formed of a homogenised plant material comprising: between 1 percent by weight and 65 percent by weight of non-tobacco plant particles, between 15 percent by weight and 55 percent by weight of aerosol former, between 2 percent by weight and 10 percent by weight of cellulose ether, and between 5 percent by weight and 50 percent by weight of additional cellulose.

US 4,333,484 relates to a process for producing a foamed smoking material comprising: providing an aqueous slurry of cellulosic material, adding from about 5 to 40% by weight, based on the cellulosic material, of a metal salt of an organic or inorganic acid, adding a foaming or blowing agent to the resulting slurry and casting or extruding the slurry and then drying the cast or extruded slurry under such conditions wherein the slurry is foamed during the casting or extruding step or during the drying step.

US 3 965 911 relates to a smoking mixture comprising a thermally degraded carbohydrate tobacco substitute as the essential smoke-producing fuel, alkali or alkaline earth carbonates, sodium carboxymethyl cellulose, and a protein.

WO 2021/122583 relates to an aerosol-forming substrate comprising one or both of cellulose and cellulose derivatives, an aerosol-former, tobacco, a nitrogen-containing nucleophilic compound, and a disaccharide.

WO 2020/012761 relates to a filling for an aroma cartridge, which contains a non-tobacco material and an aerosol former, in the form of a strip or a rod with a length of 10 to 70 mm and contains the aerosol former in an amount of 10 to 40% by mass, wherein said non-tobacco material is black tea or teas.

WO 2020/044179 relates to a shisha cartridge comprising a body comprising a cavity and an internal cavity surface, an aerosol-forming substrate disposed in the cavity, an absorbent carrier disposed in the cavity, and an aerosol former impregnated into the absorbent carrier, wherein the aerosol former comprises glycerine, propylene glycol, or a combination thereof and the absorbent carrier comprises refined cellulosic material.

EP 3 351 121 relates to tobacco substitute for use in a hookah apparatus comprising a dry gel flavour formulation comprising from about 55% to about 99% of a syrup comprising from about 1% to about 99% of one or more humectants and from about 1% to about 99% of at least one source of sugar, from about 1.0% to about 45% of one or more flavours, from about 5.0% to about 60% wt./wt. of one or more binder agents relative to the wrt of the syrup comprising the one or more flavours, optionally from about 0.5% to about 2.0% wt./wrt of one or more preservatives, optionally from about 0.01 % to about 10.0% wrt/wt. of one or more ingredients selected from the group consisting of a dye, a colouring agent, a preservative, and combinations thereof, and
optionally one or more of nicotine, a nicotine salt, a nicotine solution, and a tobacco extract.

CN 110236218 relates to a method of production of a homogenized tobacco material, said method comprising a step of suspending a binder in an aerosol-former to form a suspension, a step of creating a cellulose pulp from cellulose fibers and water, a step of providing a tobacco powder blend and combining the suspension of binder in aerosol-former, the cellulose pulp and the tobacco powder blend to form a slurry.

US 2021/259307 relates to a shisha cartridge comprising a body defining a cavity and an internal cavity surface, an aerosol-forming substrate disposed in the cavity, and a layer of gel disposed in the cavity adjacent the internal cavity surface and adjacent the aerosol-forming substrate, wherein the gel comprises 10 wt.% to 80 wt.% of an aerosol former comprising glycerine, propylene glycol, or a combination thereof and 0.2 wt.% to 10 wt.% of a gelling agent.

DE 20 2020 002254U1 discloses a moistened carrier material for use in a shisha, containing 15-25% fibers made from cellulose, cotton, cellulose acetate, grass, hemp, and/or bamboo and 75 to 85 wt.% of a liquid composition containing 50 to 90 wt.% glycerin, 5 to 25 wt.% water, 0 to 30 wt.% propylene glycol, wherein the carrier additionally contains flavorings, vitamins, CBD, tobacco flavors and / or nicotine.

Typically, traditional water pipes are used in combination with a substrate, sometimes referred to in that art as hookah tobacco, tobacco molasses, or simply as molasses. Traditional shisha substrates are relatively high in sugar (in some cases, up to -50% vs. the -20% typically found in conventional tobacco substrates, such as in combustible cigarettes). The tobacco used in shisha devices may be mixed with other ingredients to, for example, increase the volume of the vapor and smoke produced, to alter flavour, or both.

Products very similar to shisha, are the electronic cigarette and the "shisha pen". These are electronic devices which contain a liquid similar in composition to liquids used for tobacco shisha. However, the ratios are significantly different. An electronic cigarette typically contains mostly aerosol generating agent to which a small amount of nicotine and flavour are being added. The term shisha pen usually refers to the same product, but without the nicotine. These products may or may not contain sugar.

Alternatives for tobacco in shisha can be seen as a combination of a substrate, and a liquid. The currently most used non-tobacco shisha alternatives in the market are, for example, herbal shisha, i.e. basically shisha in which the tobacco leaves are replaced by dried herbs, shisha stones, i.e. stones, or pebbles from a porous minerals like zeolite, e.g. "steam stones" made from volcanic rock, and gel cubes and gel pastes, i.e. premade gels consisting of humectants formed into a gel structure (see US 2018/0199617). On the market there is also paper based shisha, i.e. a paper material impregnated with shisha liquids.

A disadvantage of herbal shisha is that still plant leaves are being consumed. Several studies have shown that the health risk of herbal shisha is the same, or greater than that of shisha tobacco smoking. A disadvantage of steam stones is not only the mass of the substrate (stone) that is high compared to the liquid, but the high heat capacity of the stones as well. It takes a long time to heat the stones before consumption can start. Also, low vapor production can be seen as a drawback. Furthermore, the pores of the stones get saturated with soot from the charcoal used for the heating and may result in breakdown products of the liquids. A disadvantage of the shisha gel is that the gel is sticky and thus it is not easy to fill the bowl. The result is dirty hands and fouling of the bowl after usage.

An objective of the present invention is to provide a cellulose based composition which forms an excellent basis for a hookah consumable composition.

Another objective of the present invention is to provide a cellulose based composition having a behaviour similar to tobacco or herbal material without one or more of the above discussed disadvantages of the shisha products.

Another objective of the present invention is to provide a cellulose based composition as a material for use as a component in the manufacture of smoking products.

### STATEMENTS OF THE INVENTION

The present invention thus provides in a first aspect a method for preparing a hookah consumable composition as defined in claim 1.

On basis of the above method one or more objects are achieved. The present inventors found that amount of aerosol generating agent in the composition of a) is limited due the subsequent step of shredding. If the amount of aerosol generating agent is too high, shredding of the composition is difficult. From a view point of durability of the hookah consumable composition, i.e. the smoke duration of a consumer, it is desirable to have a high content of aerosol generating agent in the shredded material and to reach the final content of aerosol generating agent by adding an additional amount of aerosol generating agent in the mixture of step c) thereby further increasing the amount of aerosol generating agent in the final hookah consumable composition.

In an embodiment where the present composition only consists of i) and ii) and iii), it is clear that the total amount of these components taken together must meet 100%. The person skilled in the art is able to choose the correct amount of each component within the disclosed range to arrive at the total sum of 100%. In addition, if the present composition comprises additional components, the total amount of all these components taken together must meet 100%. And in such an embodiment the person skilled in the art is also able to choose the correct amount of each component within the disclosed range to arrive at the total sum of 100%.

In the description the term "a composition" also includes equivalent terms such as "a mixture" or "a carrier material."

In an example the composition may further comprise iv) 1 to 80 wt.% of fibrous cellulose, wherein the wt.% is based on the total weight of the composition and the total amount of components taken together is 100%.

In an example the composition may further comprise 0,01 to 40 wt.% of a sweetening component, chosen from the group of natural sugar and synthetic sweetener, or a combination thereof, wherein the wt.% is based on the total weight of the composition and the total amount of components taken together is 100%.

The present inventors found a cellulose based composition which is an excellent basis for a hookah consumable composition. The present inventors found that the high absorbing effect of the composition is achieved by using a specific type of cellulose, i.e. powdered cellulose integrated into the sheet.

The composition lends its structural integrity from the incorporation of binding agents and may further be improved by the addition of cellulose fibres. The binding agents, and in case fibrous cellulose, form a web to capture the cellulose powder. Although fibrous cellulose also contributes to the absorption of glycerol in the sheet, and that it is possible to manufacture a composition as described above, where the cellulose consists only of fibrous cellulose, this material tends to bind less liquid. A further disadvantage of fibrous cellulose is that it strongly reduces the flowability of the slurry which has to be prepared for casting. Because of that, higher contents of fibrous cellulose, result in a lower solids content of said slurry, which strongly increases the processing cost. This can be overcome by using a combination of powdered cellulose and fibrous cellulose, until the desired combination of mechanical strength and absorbing properties has been achieved.

In an example the sweetening component may also comprise a synthetic sweetener as will be discussed later. The relevant ratio of such a synthetic sweetener may be calculated from the relative sweetness scale which is a common scale in this field.

The composition is a solid material that is preferably produced in the form of a sheet and the sheet in that form may already be used as a carrier material.

The present inventors surprisingly found that preloading the composition upon manufacturing with liquid components (e.g. glycerol and sugar) improves the binding of these components in the composition. As a result of this improved binding, the release rate of the volatilized components is reduced, leading to a more homogenous release over time, and prolonged consumption sessions.

In the composition an aerosol generating agent is incorporated into the sheet.. Up to 85 wt.% of aerosol generating agent may be incorporated. The aerosol generating agent is chosen from any of the following groups:
- the group of polyols with a boiling point between 150 °C and 350 °C, such as glycerol, propylene glycol, diethylene glycol, triethylene glycol and 1,3 butanediol,
- the group of esters commonly used for flavouring of food and beverages, which esters have a boiling point between 150 and 350 C such as ethyl vanillate, ethyl laurate, benzyl benzoate ,
- the group of esters of glycerol, having a boiling point between 150 and 350 C such as, diacetin, triacetin, tributyrin
- the group of organic acids, having a boiling point between 150 and 350 C, such as dodecanoic acid, arachidic acid, propylene carbonate.

A combination of different aerosol generating agents, each chosen from any of the above groups, may be used.

The aerosol generating agent is present in a range of 5 to 85 wt.%, preferably in an amount of at least 10 wt.%, more preferably at least 20 wt.%, even more preferably at least 30 wt.% and preferably in an amount of at most 85 wt.%, more preferably at most 65 wt.%, even more preferably at most 55 wt.%, wherein the wt.% is based on the total weight of the composition and the total amount of components taken together is 100%. Examples of ranges for the aerosol generating agent are 5 - 85 wt.%, preferably 10 - 65 wt.%, more preferably 20 - 55 wt.%, even more preferably 30 - 55 wt.%, wherein the wt.% is based on the total weight of the composition and the total amount of components taken together is 100%. In a preferred composition the aerosol generating agent comprises glycerol, optionally in combination with propylene glycol.

In an example the composition further comprises v) 1 to15 wt.% of an aroma, wherein the wt.% is based on the total weight of the composition and the total amount of components taken together is 100%. The aroma is preferably chosen from the group of naturally occurring aromas and synthetic aromas, especially aromas used for food preparation. Suitable aromas or flavourings include, but are not limited to, natural or synthetic menthol, peppermint, spearmint, coffee, tea, spices (such as cinnamon, clove, ginger, or combination thereof), cocoa, vanilla, fruit flavours, chocolate, eucalyptus, geranium, eugenol, agave, juniper, anethole, linalool, and any combination thereof.

In order to achieve a good structural integrity of the composition, and potentially to be able to form a sheet, the composition contains a binding agent in a range between 2% and 25 wt.%, preferably an amount of at least 3 wt.% and an amount of at most 20 wt.%, preferably at most 15 wt.%, even more preferably at most 10 wt.%, wherein the wt.% is based on the total weight of the composition and the total amount of components taken together is 100%. In an example the binding agent is selected from the group of natural binding agents, such as guar, alginate, or selected from the group of cellulose derived binding agents, such a methyl cellulose, carboxy methyl cellulose (CMC).

Furthermore, to increase tensile strength the amount of fibrous cellulose in the present composition is preferably in a range of 1 - 30 wt.%, more preferably an amount of at least 3 wt.% and more preferably at most 15 wt.%, even more preferably an amount of at most 12 wt.%, wherein the wt.% is based on the total weight of the composition, and the total amount of components taken together is 100%.

To promote the absorption of the aerosol generating agent, powdered cellulose is preferably added in an amount of at least 15 wt.%, more preferably at least 30 wt.% and even more preferably at least 40 wt.% and preferably in an amount of at most 80 wt.%, more preferably at most 70 wt.%, even more preferably at most 65 wt.%, wherein the wt.% is based on the total weight of the composition, and the total amount of components taken together is 100%.

The ratios between binding agents, fibrous cellulose, powdered cellulose, and aerosol generating agent are chosen to optimize the absorption of aerosol generating agent, and at the same time to achieve acceptable mechanical properties for the composition. It is to be noted that the total amount of all components taken together is 100%.

In an example the binding agent is thus chosen from the group of natural binding agents and cellulose-ethers, fibrous cellulose is added to further increase the tensile strength, powdered cellulose is added to absorb and bind the aerosol generating agent, and aerosol generating agent is added in an extent sufficient to generate an aerosol without combusting the composition.

In another example the composition further comprises vi) 1-15 wt.% of a humectant. The humectant is preferably chosen from the group of glycerol, propylene glycol, diethylene glycol, triethylene glycol, tetraethylene glycol, 1,3 butanediol and sorbitol, or a combination thereof. The glycerol in the composition serves as an aerosol precursor and facilitates formation of a visible aerosol.

The fibrous cellulose or cellulose fibers used for the composition is kraft pulp, or sulphate cellulose. The fibers may be refined up to between 30 and 100 SR (Schopper Riegler). Either hardwood or softwood may be used. Both bleached and unbleached kraft are suitable, but acceptable mechanical results have been achieved with bleached softwood kraft. Unbleached kraft may contain impurities that affect taste.

The Schopper-Riegler test quickly provides an idea of the degree of refining that is related to the drainage rate of a dilute pulp suspension. An applicable standard for Schopper-Riegler test is a test method according to ISO 5267/1.

The powdered cellulose used for the composition is generally a dry ground bleached cellulose. The material is known as for instance powdered cellulose, ground cellulose, micronized cellulose et cetera. Typically, the powdered cellulose has a cellulose content of 99%. The particle dimensions may vary, but acceptable results were achieved by the inventor using a powdered cellulose with a particle dimension of an average length of 60 µm, and an average cross dimension of 20 µm. Smaller particle sizes result in a more compact and dense composition, whereas larger particle sizes increasingly inhibit the flowability of the slurry required for casting, leading to lower solids contents, and increasing drying cost when producing the composition in sheet form.

In an example, the composition contains a sweetener or a sugar component.

In an example the sweetener is chosen from the group of natural sugars, i.e. pure sugar, such as invert sugar, saccharose, lactose, galactose, maltose, trehalose, allulose, sugar products, such as caster sugar, cane sugar, brown sugar, and molasses. The amount of natural sugar is preferably in a range of 5 to 40 wt.%, wherein the wt.% is based on the total weight of the composition and the total amount of components taken together is 100%.

In an example the sweetener is a synthetic sweetener, chosen from the group of aspartame, saccharin, sucralose, cyclamate, acesulfame and stevia, or a combination thereof. By using the Relative Sweetness Scale, wherein the degree of sweetness for sucrose = 1, the rating for saccharin is 300 X, for cyclamate is 30 X, for aspartame is 180 X, for acesulfame is 200 X, and for sucralose 600 X. This means that for example sucralose is sweet with 600 times as great as sucrose. The amount of synthetic sweetener is preferably in a range of 0.01 to 5 wt.%, wherein the wt.% is based on the total weight of the composition and the total amount of components taken together is 100%. The synthetic sweetener may partly or wholly replace the natural sugars.

According to the present method the composition provided in a) is prepared according to a method comprising the following steps:
A1) preparing an aqueous viscous slurry of the components i)-iii),
A2) casting the slurry of A1) as a thin layer on a support;
A3) reducing the moisture content of the aqueous viscous slurry of A2) by application of heat and/or hot air;
A4) removing the thus formed dried solid material of A3) from the support for obtaining the composition.

According to an example the shredding step b) is carried out in such a way that strips of composition having the following dimensions are obtained:
a width ranging from about 1 to 5 mm, preferably at least 1 mm, preferably at least 1.5 mm and at most 3 mm, preferable at most 2.2 mm, and
a length ranging from about 10 to about 30 mm, preferably at least 15 mm and at most 25 mm, wherein the strips of composition are preferably in a range of 50 - 250 g/m².

In an example of the present method step c) comprises a step of preparing a premix of one or more additional components chosen from the group of aerosol generating agents, synthetic sweeteners, natural sugars, and aromas and mixing the thus prepared premix with the shredded composition for obtaining the hookah consumable composition.

According to an example the step of preparing the premix comprises a step of heating a mixture comprising 10 to 40 wt.% sucrose and 60 to 90 wt.% glycerol to a temperature of about 120°C, wherein the wt.% is based on the total weight of the mixture and the total amount of components taken together is 100%. After the heating step the heated mixture may be cooled to room temperature for further processing. In an example the mixture further comprises 1 to15 wt.% aromas, wherein the wt.% is based on the total weight of the mixture and the total amount of components taken together is 100%.

In an example of the present method the mixture further comprises 5 - 15 wt.% aromas, wherein the wt.% is based on the total weight of the mixture and the total amount of components taken together is 100%.

The present invention also provides the use of a hookah consumable composition obtained according to a method as discussed above in a heating device configured to heat the hookah consumable composition to an extent sufficient to generate an aerosol without combusting the hookah consumable composition.

Reference will now be made to the examples, which depict one or more embodiments described in this disclosure.

### Example 1 (all % are wt.%, based on the total weight)

| Component | Amount (wt.%) |
|---|---|
| Cellulose fibers | 10% |
| Carboxymethylcellulose | 10% |
| Glycerine | 35% |
| Powdered cellulose | 45% |

### Example 2(all % are wt.%, based on the total weight)

| Component | Amount (wt.%) |
|---|---|
| Cellulose fibers | 10% |
| Carboxymethylcellulose | 10% |
| Powdered cellulose | 60% |
| Glycerol | 20 % |

### Example 3 (all % are wt.%, based on the total weight)

| Component | Amount (wt.%) |
|---|---|
| Methyl-cellulose | 20% |
| Glycerol | 20% |
| Powdered cellulose | 60% |

Example 3 discloses a composition where no fibrous cellulose is used, and the structural integrity is completely formed by the binding agent

### Example 4 (all % are wt.%, based on the total weight)

| Component | Amount (wt.%) |
|---|---|
| Methyl-cellulose | 20% |
| Glycerol | 20% |
| Fibrous cellulose | 60% |

Each of the compositions according to the Examples 1-4 are manufactured by preparing an aqueous viscous slurry of the components listed, casting the slurry thus prepared as a thin layer on a support and reducing the moisture content of the aqueous viscous slurry of by application of heat and/or hot air. The final composition is obtained by removing the thus formed dried solid material of from the support.

Example 4 discloses a composition, where no powdered cellulose but fibrous cellulose is used. The absorbing property of such material is less good as a result of the lack of powdered cellulose. The present inventor has found that such material offers no improved suitability for Shisha consumption over regular writing paper.

The composition according to Examples 1-3 can be used as a basis for a shisha consumption composition. Such a composition is made by combining the composition with ingredients commonly used for shisha preparation.

A typical combination of the composition with the shisha ingredients is shown in Example 5.

### Example 5 (all % are wt.%, based on the total weight)

| Component | Amount (wt.%) |
|---|---|
| Carrier of Example 1 | 23.1 % |
| Commercially available Shisha Aroma | 5.0% |
| Glycerol | 71.9% |

The composition of Example 5 results in a glycerol level in the hookah consumable of 80.0 wt.% The inventors have found that 12 grams of this composition is sufficient to fill a typical home-use hookah device, and will result in a smoking session of approximately 45 minutes. This is in line with the by consumers expected average duration of a hookah session.

When the aroma is replaced by glycerol, a glycerol level of 85 wt.% may be achieved. This will lead to a neutral tasting material. The inventors have furthermore found that when the carrier is combined with glycerol in an amount whereby 85 wt.% in the finished composition is exceeded, this excess amount of glycerol is not bound by carrier material. The composition will start to drip, the excess amount of glycerol will be lost, and does no longer contribute to the consumption

A different combination of composition suitable for hookah consumption can be prepared as follows:

### Example 6 (all % are wt.%, based on the total weight)

| Component | Amount (wt.%) |
|---|---|
| Carrier of Example 2 | 85% |
| Glycerin | 10% |
| Commercially available Shisha Aroma | 5% |

The composition of Example 6 will result in a hookah consumable containing 27% of glycerol. As with Example 5, about 12 grams of this composition is suitable for a typical home use hookah bowl. The duration of the session with this composition, however, is reduced to about 15 to 18 minutes. This is below the minimum acceptable duration for a consumer, which is about 20 minutes. This composition is therefore not suitable for a commercial application.

The compositions mentioned in Examples 5 and 6 are prepared by a step of shredding the mentioned carrier material and then mixing the shredded composition with the other components (glycerol and aroma) in the ratios as shown.

For the consumption of the material like the compositions shown in Example 5 and Example 6 in a water pipe the material must be placed in a bowl of a hookah or similar device. The method of packing is of great importance for the amount and consistency of aerosol generated. If the packing is too dense, the hot air can't pass through the material well. This leads to a strong draw resistance, and "channeling". When channeling occurs, the air passes through a limited number of channels in the packing, and therefore the material is not completely used. Is the packing too fluffy, then upon consumption the aerosol generating material expands, with an increased risk of the material touching the heating element and charring. This charring leads to an unwanted taste.

The present inventors found that when the composition according to any of the Examples 1 to 4 is present in sheet form, optimal dimensions for the material exist. The optimal dimensions for the sheet form composition are as follows:

| | |
|---|---|
| Width: | 1 to 5 mm, preferably about 2 mm |
| Length: | 10 to 30 mm, preferably about 20 mm. |

A smaller width, i.e. a width below 1 mm, will lead to a more compact packing in the Shisha bowl. The same applies for a length below 10 mm. The present inventors found that a sheet like composition having a larger width (i.e. larger than about 5mm) and/or length (i.e. larger than about 30mm) will lead to too open structure of the packing, which promotes rapid evaporation, expansion of the packing, and potentially the packing touching the heating element, leading to burning of the material.

In practice one may shredder the sheet like composition with a device that is the same device as or similar to an office paper shredder. The shredded material may then be mixed with additional amounts of aroma, sweetener and aerosol generating agent. The mixed material is ready for consumption.

When preparing a shisha composition, a composition is mixed with a liquid. An example of such a liquid is a combination of glycerol and a sugar containing component. An example of such a sugar containing component is honey, or even an invert sugar may be used. Caster sugar is typically not being used [in shisha], as it does not dissolve in glycerol. However, the present inventor found that a liquid mixture of glycerol and caster sugar is obtained when glycerol and caster sugar are mixed at a temperature of about 120 °C. Even at a concentration of about 25 wt.% caster sugar, based on the total weight of the mixture, this mixture remains liquid at room temperature, and even at a temperature of about 7 °C.

Without wishing to be bound by theory, it is believed that at this temperature, the sucrose, i.e. the caster sugar composition, is split into its mono sugars glucose and fructose. This is a well-known chemical reaction, i.e. hydrolysis of sugar, but this hydrolysis reaction normally requires the presence of water molecules. The water concentration of the glycerol used in these experiments is only about 0.3 wt.% of water, which concentration is not enough to hydrolyze the amount of sucrose in the mixture. The inventor assumes that the OH groups of the glycerol perform the same function as that of the water normally used, and/or that glycerol serves as a donor of the water normally required for hydrolysis.

## Claims

1. A method for preparing a hookah consumable composition, the method comprising the following steps:
a) providing a composition, comprising:
i) 2 to 25 wt.% of one or more binding agents;
ii) 5 to 85 wt.% of an aerosol generating agent, and
iii) 10 to 80 wt.% of powdered cellulose;
wherein the wt.% is based on the total weight of the composition, and the total amount of components taken together is 100%, wherein the composition provided in a) is prepared according to a method comprising the following steps:
A1) preparing an aqueous viscous slurry of the components i)-iii),
A2) casting the slurry of A1) as a thin layer on a support;
A3) reducing the moisture content of the aqueous viscous slurry of A2) by application of heat and/or hot air;
A4) removing the thus formed dried solid material of A3) from the support for obtaining the composition,
b) shredding the composition of a),
c) providing one or more additional components chosen from the group of aerosol generating agents, synthetic sweeteners, natural sugars, and aromas,
d) mixing the shredded composition of b) with one or more additional components of c) for obtaining the hookah consumable composition,
wherein step d) is carried out in such a way that the total amount of aerosol generating agents in the hookah consumable composition thus obtained is in a range of 30 - 85 wt.%, based on the total weight of the hookah consumable composition.

2. A method according to claim 1, wherein shredding step b) is carried out in such a way that strips of composition having the following dimensions are obtained:
a width ranging from about 1 to 5 mm, preferably at least 1 mm, preferably at least 1.5 mm and at most 3 mm, preferable at most 2.2 mm, and
a length ranging from about 10 to about 30 mm, preferably at least 15 mm and at most 25 mm.

3. A method according to claim 2, wherein the strips of composition are in a range of 50 - 250 g/m².

4. A method according to any one or more of claims 1-3, wherein step c) comprises a step of preparing a premix of one or more additional components chosen from the group of aerosol generating agents, synthetic sweeteners, natural sugars, and aromas and mixing the thus prepared premix with the shredded composition for obtaining the hookah consumable composition.

5. A method according to claim 4, wherein the step of preparing the premix comprises a step of heating a mixture comprising 10 to 40 wt.% sucrose and 60 to 90 wt.% glycerol to a temperature of about 120 °C, wherein the wt.% is based on the total weight of the mixture and the total amount of components taken together is 100%.

6. A method according to claim 5, wherein the mixture further comprises 5 - 15 wt.% aromas, wherein the wt.% is based on the total weight of the mixture and the total amount of components taken together is 100%.

7. A method according to any one or more of claims 1-6, wherein the composition further comprises:
iv) 1 to 80 wt.% of fibrous cellulose, wherein the wt.% is based on the total weight of the composition, and the total amount of components taken together is 100%.

8. A method according to any one or more of claims 1-7, wherein the composition further comprises:
v) 0,01 to 40 wt.% of a sweetening component, chosen from the group of natural sugar and synthetic sweetener, or a combination thereof, wherein the wt.% is based on the total weight of the composition, and the total amount of components taken together is 100%.

9. A method according to any one or more of claims 1-8, wherein the composition further comprises:
vi) 1 to 15 wt.% of one or more aromas, wherein the wt.% is based on the total weight of the composition, and the total amount of components taken together is 100%.

10. A method according to any one or more of the preceding claims, wherein the amount of powdered cellulose iii) is at least 15 wt.%, preferably at least 30 wt.%, more preferably at least 40 wt.% and at most 80 wt.%, preferably at most 70 wt.%, more preferably at most 65 wt.%, wherein the wt.% is based on the total weight of the composition, and the total amount of components taken together is 100%.

11. A method according to any one or more of the preceding claims, wherein the amount of aerosol generating agent ii) is at least 5 wt.%, preferably at least 10 wt.%, more preferably at least 20 wt.%, even more preferably at least 30 wt.% and at most 85 wt.%, preferably at most 65 wt.% and more preferably at most 55 wt.%, wherein the wt.% is based on the total weight of the composition, and the total amount of components taken together is 100%.

12. A method according to any one or more of claims 8-11, wherein the natural sugar is chosen from the group of pure sugar, such as invert sugar, saccharose, lactose, galactose, maltose, trehalose, allulose, sugar products, such as caster sugar, cane sugar, browns sugar and molasses, or a combination thereof, preferably in an amount of 5 to 40 wt.%, wherein the wt.% is based on the total weight of the composition and the total amount of components taken together is 100%.

13. A method according to any one or more of claims 8-11, wherein the synthetic sweetener is chosen from the group of aspartame, saccharin, sucralose, cyclamate, acesulfame and stevia, or a combination thereof, preferably in an amount of 0.01 to 5 wt.%, wherein the wt.% is based on the total weight of the composition and the total amount of components taken together is 100%.

14. The use of a hookah consumable composition obtained according to a method according to any one or more of claims 1-13 in a heating device configured to heat the hookah consumable composition to an extent sufficient to generate an aerosol without combusting the hookah consumable composition.

## Patentansprüche

1. Verfahren zur Herstellung einer Huka-Verbrauchszusammensetzung, wobei das Verfahren die folgenden Schritte umfasst:
a) Bereitstellen einer Zusammensetzung umfassend:
i) 2 bis 25 Gew.-% an einem oder mehreren Bindemitteln;
ii) 5 bis 85 Gew.-% an einem aerosolerzeugenden Mittel; und
iii) 10 bis 80 Gew.-% pulverförmige Cellulose;
wobei die Gew.-% auf das Gesamtgewicht der Zusammensetzung bezogen sind und die Gesamtmenge der Komponenten zusammengenommen 100 % beträgt, wobei die bei a) bereitgestellte Zusammensetzung gemäß einem Verfahren hergestellt ist, das die folgenden Schritte umfasst:
A1) Herstellen einer wässrigen viskosen Aufschlämmung der Komponenten i)-iii),
A2) Gießen der Aufschlämmung von A1) als dünne Schicht auf einen Träger;
A3) Verringern des Feuchtegehalts der wässrigen viskosen Aufschlämmung von A2) durch Anwenden von Wärme und/oder heißer Luft;
A4) Entfernen des so gebildeten getrockneten festen Materials von A3) von dem Träger, um die Zusammensetzung zu erhalten,
b) Zerkleinern der Zusammensetzung von a),
c) Bereitstellen einer oder mehrerer zusätzlicher Komponenten ausgewählt aus der Gruppe von aerosolerzeugenden Mitteln, synthetischen Süßstoffen, natürlichen Zuckern und Aromen,
d) Mischen der zerkleinerten Zusammensetzung von b) mit einer oder mehreren zusätzlichen Komponenten von c), um die Huka-Verbrauchszusammensetzung zu erhalten,
wobei Schritt d) so durchgeführt wird, dass die Gesamtmenge an aerosolerzeugenden Mitteln in der erhaltenen Huka-Verbrauchszusammensetzung in einem Bereich von 30-85 Gew.-%, bezogen auf das Gesamtgewicht der Huka-Verbrauchszusammensetzung, liegt.

2. Verfahren gemäß Anspruch 1, wobei Zerkleinern bei Schritt b) so durchgeführt wird, dass Streifen von Zusammensetzung mit den folgenden Abmessungen erhalten werden:
eine Breite in dem Bereich von etwa 1 bis 5 mm, vorzugsweise wenigstens 1 mm, vorzugsweise wenigstens 1,5 mm und höchstens 3 mm, vorzugsweise höchstens 2,2 mm, und
eine Länge in dem Bereich von etwa 10 bis etwa 30 mm, vorzugsweise wenigstens 15 mm und höchstens 25 mm.

3. Verfahren gemäß Anspruch 2, wobei die Streifen von Zusammensetzung in einem Bereich von 50-250 g/m² liegen.

4. Verfahren gemäß einem oder mehreren der Ansprüche 1-3, wobei Schritt c) einen Schritt des Herstellens einer Vormischung von einer oder mehreren zusätzlichen Komponenten ausgewählt aus der Gruppe von aerosolerzeugenden Mitteln, synthetischen Süßstoffen, natürlichen Zuckern und Aromen und Mischen der so hergestellten Vormischung mit der zerkleinerten Zusammensetzung umfasst, um die Huka-Verbrauchszusammensetzung zu erhalten.

5. Verfahren gemäß Anspruch 4, wobei der Schritt des Herstellens der Vormischung einen Schritt des Erhitzens eines Gemischs umfassend 10 bis 40 Gew.- % Saccharose und 60 bis 90 Gew.-% Glycerol auf eine Temperatur von etwa 120 °C umfasst, wobei die Gew.-% auf das Gesamtgewicht des Gemischs bezogen sind und die Gesamtmenge der Komponenten zusammengenommen 100 % beträgt.

6. Verfahren gemäß Anspruch 5, wobei das Gemisch ferner 5-15 Gew.-% Aromen umfasst, wobei die Gew.-% auf das Gesamtgewicht des Gemischs bezogen sind und die Gesamtmenge der Komponenten zusammengenommen 100 % beträgt.

7. Verfahren gemäß einem oder mehreren der Ansprüche 1-6, wobei die Zusammensetzung ferner umfasst:
iv) 1 bis 80 Gew.-% an faserartiger Cellulose, wobei die Gew.-% auf das Gesamtgewicht des Gemischs bezogen sind und die Gesamtmenge der Komponenten zusammengenommen 100 % beträgt.

8. Verfahren gemäß einem oder mehreren der Ansprüche 1-7, wobei die Zusammensetzung ferner umfasst:
v) 0,01 bis 40 Gew.-% an einer Süßungskomponente ausgewählt aus der Gruppe von natürlichem Zucker und synthetischem Süßstoff oder einer Kombination davon, wobei die Gew.-% auf das Gesamtgewicht des Gemischs bezogen sind und die Gesamtmenge der Komponenten zusammengenommen 100 % beträgt.

9. Verfahren gemäß einem oder mehreren der Ansprüche 1-8, wobei die Zusammensetzung ferner umfasst:
vi) 1 bis 15 Gew.-% an einem oder mehreren Aromen, wobei die Gew.-% auf das Gesamtgewicht des Gemischs bezogen sind und die Gesamtmenge der Komponenten zusammengenommen 100 % beträgt.

10. Verfahren gemäß einem oder mehreren der vorstehenden Ansprüche, wobei die Menge an pulverförmiger Cellulose iii) wenigstens 15 Gew.-%, vorzugsweise wenigstens 30 Gew.-%, bevorzugter wenigstens 40 Gew.-%, und höchstens 80 Gew.- %, vorzugsweise höchstens 70 Gew.-%, bevorzugter höchstens 65 Gew.-% beträgt, wobei die Gew.-% auf das Gesamtgewicht des Gemischs bezogen sind und die Gesamtmenge der Komponenten zusammengenommen 100 % beträgt.

11. Verfahren gemäß einem oder mehreren der vorstehenden Ansprüche, wobei die Menge an aerosolerzeugendem Mittel ii) wenigstens 5 Gew.-%, vorzugsweise wenigstens 10 Gew.-%, bevorzugter wenigstens 20 Gew.-%, noch bevorzugter wenigstens 30 Gew.-%, und höchstens 85 Gew.-%, vorzugsweise höchstens 65 Gew.-% und bevorzugter höchstens 55 Gew.-% beträgt, wobei die Gew.- % auf das Gesamtgewicht des Gemischs bezogen sind und die Gesamtmenge der Komponenten zusammengenommen 100 % beträgt.

12. Verfahren gemäß einem oder mehreren der Ansprüche 8-11, wobei der natürliche Zucker ausgewählt ist aus der Gruppe von reinem Zucker, wie z.B. Invertzucker, Saccharose, Lactose, Galactose, Maltose, Trehalose, Allulose, Zuckerprodukten, wie z.B. Puderzucker, Rohrzucker, brauner Zuckern und Molassen, oder einer Kombination davon, vorzugsweise in einer Menge von 5 bis 40 Gew.-%, wobei die Gew.-% auf das Gesamtgewicht des Gemischs bezogen sind und die Gesamtmenge der Komponenten zusammengenommen 100 % beträgt.

13. Verfahren gemäß einem oder mehreren der Ansprüche 8-11, wobei der synthetische Süßstoff ausgewählt ist aus der Gruppe von Aspartam, Saccharin, Sucralose, Cyclamat, Acesulfam und Stevia oder einer Kombination davon, vorzugsweise in einer Menge von 0,01 bis 5 Gew.-%, wobei die Gew.-% auf das Gesamtgewicht des Gemischs bezogen sind und die Gesamtmenge der Komponenten zusammengenommen 100 % beträgt.

14. Verwendung einer Huka-Verbrauchszusammensetzung, erhalten gemäß einem oder mehreren der Ansprüche 1-13, in einer Heizvorrichtung, gestaltet zum Erhitzen der Huka-Verbrauchszusammensetzung zu einem Maß, das ausreicht, um ohne Verbrennung der Huka-Verbrauchszusammensetzung ein Aerosol zu erzeugen.

## Revendications

1. Procédé de préparation d'une composition consommable de narguilé, le procédé comprenant les étapes suivantes :
a) la fourniture d'une composition, comprenant :
i) 2 à 25% en poids d'un ou plusieurs agents liants ;
ii) 5 à 85% en poids d'un agent générateur d'aérosol, et
iii) 10 à 80% en poids de cellulose en poudre ;
où le % en poids est basé sur le poids total de la composition, et la quantité totale de composants pris ensemble est de 100%, où la composition fournie en a) est préparée selon un procédé comprenant les étapes suivantes :
A1) la préparation d'une suspension aqueuse visqueuse des composants i) à iii),
A2) la coulée de la suspension de A1) en couche mince sur un support ;
A3) la réduction de la teneur en humidité de la suspension aqueuse visqueuse de A2) par application de chaleur et/ou d'air chaud ;
A4) le retrait du matériau solide séché ainsi formé de A3) du support pour obtenir la composition,
b) le déchiquetage de la composition de a),
c) la fourniture d'un ou plusieurs composants supplémentaires choisis dans le groupe des agents générateurs d'aérosols, des édulcorants synthétiques, des sucres naturels et des arômes,
d) le mélange de la composition déchiquetée de b) avec un ou plusieurs composants supplémentaires de c) pour obtenir la composition consommable de narguilé,
dans lequel l'étape d) est réalisée de manière à ce que la quantité totale d'agents générateurs d'aérosols dans la composition consommable de narguilé ainsi obtenue se situe dans une plage allant de 30 à 85% en poids, par rapport au poids total de la composition consommable de narguilé.

2. Procédé selon la revendication 1, dans lequel l'étape de déchiquetage b) est réalisée de manière à obtenir des bandes de composition ayant les dimensions suivantes :
une largeur allant d'environ 1 à 5 mm, de préférence d'au moins 1 mm, de préférence d'au moins 1,5 mm et d'au plus 3 mm, de préférence d'au plus 2,2 mm, et
une longueur allant d'environ 10 à environ 30 mm, de préférence d'au moins 15 mm et d'au plus 25 mm.

3. Procédé selon la revendication 2, dans lequel les bandes de composition se situent dans une plage allant de 50 à 250 g/m².

4. Procédé selon l'une quelconque ou plusieurs des revendications 1 à 3, dans lequel l'étape c) comprend une étape de préparation d'un prémélange d'un ou plusieurs composants supplémentaires choisis dans le groupe des agents générateurs d'aérosols, des édulcorants synthétiques, des sucres naturels et des arômes et de mélange du prémélange ainsi préparé avec la composition déchiquetée pour obtenir la composition consommable de narguilé.

5. Procédé selon la revendication 4, dans lequel l'étape de préparation du prémélange comprend une étape de chauffage d'un mélange comprenant 10 à 40% en poids de saccharose et 60 à 90% en poids de glycérol à une température d'environ 120°C, dans lequel le % en poids est basé sur le poids total du mélange et la quantité totale des composants pris ensemble est de 100%.

6. Procédé selon la revendication 5, dans lequel le mélange comprend en outre 5 à 15% en poids d'arômes, dans lequel le % en poids est basé sur le poids total du mélange et la quantité totale des composants pris ensemble est de 100%.

7. Procédé selon l'une quelconque ou plusieurs des revendications 1 à 6, dans lequel la composition comprend en outre :
iv) 1 à 80% en poids de cellulose fibreuse, où le % en poids est basé sur le poids total de la composition, et la quantité totale des composants pris ensemble est de 100%.

8. Procédé selon l'une quelconque ou plusieurs des revendications 1 à 7, dans lequel la composition comprend en outre :
v) 0,01 à 40% en poids d'un composant édulcorant, choisi dans le groupe constitué du sucre naturel et d'un édulcorant synthétique, ou une combinaison de ceux-ci, où le % en poids est basé sur le poids total de la composition, et la quantité totale des composants pris ensemble est de 100%.

9. Procédé selon l'une quelconque ou plusieurs des revendications 1 à 8, dans lequel la composition comprend en outre :
vi) 1 à 15% en poids d'un ou plusieurs arômes, où le % en poids est basé sur le poids total de la composition, et la quantité totale des composants pris ensemble est de 100%.

10. Procédé selon l'une quelconque ou plusieurs des revendications précédentes, dans lequel la quantité de cellulose en poudre iii) est d'au moins 15% en poids, de préférence d'au moins 30% en poids, plus préférablement d'au moins 40% en poids et d'au plus 80% en poids, de préférence d'au plus 70% en poids, plus préférablement d'au plus 65% en poids, où le % en poids est basé sur le poids total de la composition, et la quantité totale des composants pris ensemble est de 100%.

11. Procédé selon l'une quelconque ou plusieurs des revendications précédentes, dans lequel la quantité d'agent générateur d'aérosol ii) est d'au moins 5% en poids, de préférence d'au moins 10% en poids, plus préférablement d'au moins 20% en poids, encore plus préférablement d'au moins 30% en poids et d'au plus 85% en poids, de préférence d'au plus 65% en poids et plus préférablement d'au plus 55% en poids, dans lequel le % en poids est basé sur le poids total de la composition, et la quantité totale des composants pris ensemble est de 100%.

12. Procédé selon l'une quelconque ou plusieurs des revendications 8 à 11, dans lequel le sucre naturel est choisi dans le groupe du sucre pur, tel que le sucre inverti, le saccharose, le lactose, le galactose, le maltose, le tréhalose, l'allulose, des produits sucrés, tels que le sucre en poudre, le sucre de canne, le sucre brun et la mélasse, ou une combinaison de ceux-ci, de préférence en une quantité de 5 à 40% en poids, où le % en poids est basé sur le poids total de la composition et la quantité totale des composants pris ensemble est de 100%.

13. Procédé selon l'une quelconque ou plusieurs des revendications 8 à 11, dans lequel l'édulcorant synthétique est choisi dans le groupe de l'aspartame, de la saccharine, du sucralose, du cyclamate, de l'acésulfame et de la stévia, ou une combinaison de ceux-ci, de préférence en une quantité de 0,01 à 5% en poids, où le % en poids est basé sur le poids total de la composition et la quantité totale des composants pris ensemble est de 100%.

14. Utilisation d'une composition consommable de narguilé obtenue selon un procédé selon l'une quelconque ou plusieurs des revendications 1 à 13 dans un dispositif de chauffage configuré pour chauffer la composition consommable de narguilé à un degré suffisant pour générer un aérosol sans brûler la composition consommable de narguilé.
